

## UNITED STATES PATENT OFFICE.

JOHN W. LITTLEFORD, OF ALAMEDA, CALIFORNIA, ASSIGNOR TO MINERALS SEPARATION NORTH AMERICAN CORPORATION, OF NEW YORK, N. Y., A CORPORATION OF MARYLAND.

## ORE CONCENTRATION.

No Drawing.

Application filed April 5, 1922. Serial No. 549,878.

This invention relates to the froth-flootation concentration of ores and is herein disclosed as involving in suitable admixture, the use of asphalts, asphaltites or pyrogenous asphalts as mineral-frothing agents. I have discovered that certain classes of hydrocarbons used in certain combinations may be used very effectively as mineral-frothing agents with a great many ores, either with or without mineral-frothing agents of hitherto recognized types. I have found that with many ores substantially the same results are obtained by using, as mineral-frothing agents, various materials such as the asphaltite gilsonite or the lake asphalts or the pyrogenous asphalts known as air-blown asphalts, when mixed or carried in or dissolved in hydrocarbons of the benzene series, and I generally use what seems to be a concentrated solution of the asphalt. The air-blown asphalt appears to be equally effective whether made from paraffin-base hydrocarbons or asphaltic-base hydrocarbons. The carrier for the asphalt as indicated above, is advantageously a hydrocarbon of the benzene series such as xylol, but a mixture of hydrocarbons of the benzene series when used as a carrier seems to produce a more effective frothing agent than would be supposed from a comparison of the individual hydrocarbons when used separately as such carriers for the asphalt. Commercial xylol is such a mixture, and coal-tar naphtha largely consists of such a mixture.

In concentrating many ores it is found advantageous to add carbonate of soda or a small amount of pine oil or other mineral-frothing agents or both substances. Carbonate of soda also has the effect of increasing the differential action in selecting certain normally floatable minerals over others when used in combination with benzene-series hydrocarbons carrying the above described asphalt with or without another or other mineral-frothing agents.

It has been found that a frothing agent consisting of asphalt mixed with or carried

in hydrocarbons of the benzene series, floats carbonate of lead in a lead carbonate ore without artificial sulphidization, and moreover floats the portion of the carbonate containing the silver in preference to the carbonate low in silver. A second treatment with the mixture of asphalt and benzene series hydrocarbon after sulphidization or with concomitant sulphidization will then float the remainder of the lead in the treatment of many ores. Moreover, it has been found that frequently treatment with the benzene-series hydrocarbons alone suffices for the second treatment when a first froth has been produced by the asphalt mixed with or carried in the hydrocarbons of the benzene series.

It is also possible to adjust the proportions and procedure so as to separate from a lead-zinc ore or a lead-zinc silver ore, a first concentrate containing the lead, or the lead and the silver, and low in zinc, and a second concentrate high in zinc and relatively low in silver and lead. Such a separation can also be effected in the presence of copper. If the ore also contains normally floatable iron, the relative proportions of the asphalt and benzene-series frothing agent used can often be readily adjusted so as to float first a lead concentrate and then a zinc concentrate, both low in iron and both relatively free from the other metal, frequently obtaining in the single concentrations, concentrates conforming to the severest requirements of the smelters. Sometimes a preagitation with a benzene-series hydrocarbon and asphalt frothing agent is advantageous, more of the frothing agent being added to form a froth after a suitable amount of the preliminary agitation.

The San Francisco Del Oro lead-zinc ore when agitated for ten minutes with the benzene-series hydrocarbon xylol carrying the blown asphaltic-base petroleum asphalt known as petroelastic cement, used at the rate of 0.7 pounds of mixture per ton of ore, yielded a lead concentrate, and upon further agitation for fifteen minutes, with crude sol-

vent naphtha 0.8 pounds per ton of ore, yielded a zinc concentrate. The results are shown in the following table:

| Assays.       |          |      |          |          |          |    |
|---------------|----------|------|----------|----------|----------|----|
|               | Wt.      | Ag.  | Pb.      | Zn.      | Fe.      |    |
| Heads.....    | Per cent | Oz.  | Per cent | Per cent | Per cent |    |
| Pb. conc..... | 100.0    | 24.8 | 9.4      | 19.8     | 5.5      |    |
| 20.5          | 86.5     | 40.0 | 22.0     | 7.2      |          | 70 |
| Zn. conc..... | 35.8     | 21.3 | 2.4      | 37.0     | 7.5      |    |
| Tails.....    | 43.7     | 2.3  | 0.97     | 4.6      | 3.0      |    |

Recoveries.

|               | Ag.   | Pb.   | Zn.   | Fe.   |
|---------------|-------|-------|-------|-------|
| Heads.....    | 100.0 | 100.0 | 100.0 | 100.0 |
| Pb. conc..... | 65.2  | 86.5  | 22.8  | 27.0  |
| Zn. conc..... | 30.8  | 9.0   | 67.0  | 49.1  |
| Tails.....    | 4.0   | 4.5   | 10.2  | 23.9  |

20 A lead carbonate ore from Alaska, when agitated for 18 minutes with carbonate of soda 5.0 pounds per ton, petrolastic cement carried in xylol, 2.3 pounds per ton, and sodium silicate, 1.5 pounds per ton, yielded a 25 concentrate rich in silver and carrying a large amount of lead. A second agitation for 12 minutes with sodium sulphide, 2.0 pounds per ton, and 0.5 pounds of the petrolastic-cement-xylol mixture, yielded a 30 concentrate rich in lead and poor in silver. The results are shown in the following table:

|              | Assays   |       |          | Recovery |          |
|--------------|----------|-------|----------|----------|----------|
|              | Wt.      | Ag.   | Pb.      | Ag.      | Pb.      |
| Heads.....   | Per cent | Oz.   | Per cent | Per cent | Per cent |
| Conc. A..... | 100.0    | 78.68 | 28.4     | 100.0    | 100.0    |
| 31.0         | 224.88   | 50.8  | 88.6     | 69.8     | 55.6     |
| Conc. B..... | 20.1     | 32.56 | 57.2     | 8.3      | 40.4     |
| Tails.....   | 48.9     | 12.0  | 5.5      | 3.1      | 4.0      |

40 Another sample of lead carbonate ore from a region of Alaska where transportation conditions necessitated rich concentrates, was agitated for 10 minutes with xylol carrying 45 petrolastic cement, used at the rate of 1.5 pounds per ton, to obtain a concentrate rich in silver, then sulphidized with sodium sulphide, and then agitated for twenty minutes with 0.5 pounds per ton of the same petrolastic cement to produce a concentrate rich in lead. The final froth after further agitation was collected as a middling, and the tailings were table concentrated. The results are shown in the following table:

|                 | Assays   |      |          | Recoveries |          |
|-----------------|----------|------|----------|------------|----------|
|                 | Wt.      | Ag.  | Pb.      | Ag.        | Pb.      |
| Heads.....      | Per cent | Oz.  | Per cent | Per cent   | Per cent |
| Conc. A.....    | 100.0    | 82.4 | 32.0     | 100.0      | 100.0    |
| 10.7            | 433.3    | 61.6 | 56.2     | 20.6       |          |
| Conc. B.....    | 24.2     | 88.1 | 63.6     | 23.8       | 48.0     |
| Midd. B.....    | 7.0      | 43.7 | 28.7     | 3.7        | 6.3      |
| Table conc..... | 4.5      | 27.2 | 30.6     | 1.5        | 4.3      |
| Tails.....      | 53.6     | 19.6 | 12.4     | 12.8       | 20.8     |

55 Ore from the Simon Silver Lead Co. of

Mina, Nevada, when agitated for ten minutes with soda at 5 pounds per ton, and 1.2 pounds per ton of a mixture of paraffin-base petroleum air-blown asphalt carried in xylol, yielded a silver-lead concentrate A. 70 When the remaining pulp was agitated for 17 minutes with copper sulphate, 0.3 pounds per ton, American Tar Products Co. water gas tar, 1.0 pounds per ton, cresylic acid, 0.3 pounds per ton, and 0.4 pounds per ton of the same asphalt carried in xylol, it yielded 75 a zinc concentrate B. The results are shown in the following table:

| Assays.      |          |      |          |          |          |    |
|--------------|----------|------|----------|----------|----------|----|
|              | Wt.      | Ag.  | Pb.      | Zn.      | Fe.      |    |
| Heads.....   | Per cent | Oz.  | Per cent | Per cent | Per cent |    |
| Conc. A..... | 100.0    | 3.54 | 6.73     | 6.34     | 5.54     |    |
| 0.1          | 27.1     | 51.6 | 4.6      | 3.4      |          |    |
| Conc. B..... | 13.6     | 6.67 | 7.56     | 25.6     | 8.3      |    |
| Tails.....   | 77.3     | 0.6  | 1.29     | 1.4      | 5.3      | 85 |

Per cent recovery.

|              | Ag.   | Pb.   | Zn.   | Fe.   |
|--------------|-------|-------|-------|-------|
| Heads.....   | 100.0 | 100.0 | 100.0 | 100.0 |
| Cone. A..... | 61.3  | 69.8  | 6.6   | 5.6   |
| Conc. B..... | 23.7  | 15.3  | 76.3  | 20.4  |
| Tails.....   | 12.0  | 14.9  | 17.1  | 74.0  |

Similar results were obtained on this same ore by other froth-flotation treatment, the same except for the use of petrolastic cement instead of the paraffin-base air-blown asphalt.

5 Similar results were obtained on this same ore by other froth-flotation treatment, the same except for the use of petrolastic cement instead of the paraffin-base air-blown asphalt.

Lead-zinc-iron ore from the Consolidated Mining and Smelting Co. of Trail, British Columbia, was agitated for 5 minutes with soda ash, 1.5 pounds per ton, and gilsonite carried in xylol, 0.9 pounds per ton, to yield a lead concentrate, which was further agitated for 5 minutes with 0.2 pounds per ton of the same gilsonite-xylol mixture and .02 pounds per ton of the white pine oil of the Georgia Pine Turpentine Co. to produce a final lead concentrate A and a middling A. The reject from the first concentrate was agitated for 10 minutes with sulphate of copper, 1.25 pounds per ton, and 1.0 pounds per ton of Barrett #4 coal-tar creosote, to produce a zinc concentrate. This zinc concentrate was agitated for 7 minutes with 0.3 pounds per ton of Barrett #4 coal tar creosote to produce concentrate B and middling B. 70% of the iron went into the tailings. The results are shown in the following table:

|               | Assays   |          |          | Per cent recovery |       |       |       |
|---------------|----------|----------|----------|-------------------|-------|-------|-------|
|               | Wt.      | Pb.      | Zn.      | Fe.               | Pb.   | Zn.   | Fe.   |
| Heads.....    | Per cent | Per cent | Per cent | Per cent          |       |       |       |
| Conc. A.....  | 100.0    | 8.97     | 14.88    | 34.24             | 100.0 | 100.0 | 100.0 |
| 12.75         | 54.4     | 13.0     | 6.2      | 77.3              | 11.2  | 2.3   |       |
| Midds. A..... | 2.0      | 16.2     | 13.6     | 32.6              | 3.6   | 1.8   | 1.9   |
| Concs. B..... | 29.75    | 4.8      | 41.6     | 15.2              | 16.0  | 83.2  | 13.1  |
| Midds. B..... | 8.5      | 2.0      | 4.0      | 51.6              | 1.8   | 2.3   | 12.7  |
| Tails.....    | 47.0     | 0.027    | 0.5      | 50.8              | 1.3   | 1.5   | 70.0  |

120

125

115

110

105

100

95

90

85

80

75

70

65

60

55

Substantially the same results were obtained by similar treatment with a xylol mixture in which petroelastic cement was substituted for the gilsonite, and 0.5 pounds

5 per ton of such mixture used instead of adding the white pine oil for retreating the lead concentrate.

An iron bearing lead-zinc ore from the Moulton Mining Co. of Butte, Montana, was 10 agitated 10 minutes with soda ash, 5.0 pounds per ton, and 0.7 pounds per ton of petroelastic cement carried in xylol to produce a lead concentrate. This concentrate was agitated 5 minutes with soda ash, 2.0 15 pounds per ton, and 0.3 pounds per ton petroelastic cement carried in xylol, to produce a finished concentrate and a lead middling. The reject of the first concentrate was agitated 20 minutes with heavy coal tar 20 naphtha 1.0 pounds per ton, to produce a zinc concentrate. This concentrate was re-agitated 5 minutes with 0.3 pounds per ton of heavy coal-tar naphtha to produce a finished zinc concentrate and a zinc middling. 25 40% of the iron went into the tailings but only 2% of the zinc and substantially none of the lead. The results are shown in the following table:

30 *Assays.*

|                | Wt.      | Ag.   | Cu.      | Pb.      | Zn       | Fe.      | Ins.     |
|----------------|----------|-------|----------|----------|----------|----------|----------|
|                | Per cent | Oz.   | Per cent | Per cent | Per cent | Per cent | Per cent |
| Heads.....     | 100.0    | 4.38  | 30       | 5.8      | 11.6     | 7.4      | 62.0     |
| Pb. cones..... | 6.7      | 19.56 | 0.5      | 48.0     | 11.2     | 9.7      | 1.4      |
| Pb. midds..... | 3.8      | 16.52 | 0.68     | 25.2     | 14.5     | 19.0     | —        |
| Zn. cones..... | 22.5     | 6.1   | 0.8      | 6.4      | 42.4     | 10.2     | 1.4      |
| Zn. midds..... | 5.5      | 6.53  | 0.36     | 2.6      | 13.2     | 16.0     | —        |
| Tails.....     | 61.5     | 1.16  | 0.08     | 0.0108   | 0.4      | 4.8      | —        |

40 *Per cent recovery.*

|                | Ag.   | Pb.   | Zn.   | Fe.   |
|----------------|-------|-------|-------|-------|
| Heads.....     | 100.0 | 100.0 | 100.0 | 100.0 |
| Pb. cones..... | 30.0  | 56.0  | 6.5   | 8.8   |
| Pb. midds..... | 14.4  | 16.7  | 2.7   | 9.7   |
| Zn. cones..... | 31.2  | 25.0  | 82.5  | 30.9  |
| Zn. midds..... | 8.2   | 2.3   | 6.3   | 10.5  |
| Tails.....     | 16.2  | —     | 2.0   | 40.1  |

Similar results were obtained when an air-blown paraffin-base asphalt was substituted for the petroelastic cement in the xylol mixture.

An iron bearing gold-silver-lead ore from Redding, California, was given 25 minutes 55 preagitation with sodium silicate 0.8 pounds per ton, a mixture of paraffin-base-petroleum-air-blown asphalt and xylol, 1.0 pounds per ton, and was then agitated 10 minutes with separation of a froth. This concentrate was then agitated for 15 minutes with 1.0 pound of heavy coal tar naphtha per ton of original ore to form a finished concentrate and a middling. Over 90% of the silver and lead were recovered and nearly 60 80% of the gold, while over 70% of the iron

was rejected. The results are shown in the following table:

*Assays.*

|            | Wt.      | Au.   | Ag.      | Cu.      | Pb.      | Zn.      | Fe.      | 70 |
|------------|----------|-------|----------|----------|----------|----------|----------|----|
|            | Per cent | Oz.   | Per cent | Per cent | Per cent | Per cent | Per cent | 75 |
| Heads..... | 100.0    | 0.076 | 37.9     | 0.45     | 2.19     | 1.92     | 2.38     |    |
| Cones..... | 6.5      | 0.93  | 551.0    | 5.68     | 30.4     | 22.0     | 6.7      |    |
| Midds..... | 4.5      | 0.06  | 29.6     | 0.22     | 1.02     | 4.8      | 5.6      |    |
| Tails..... | 89.0     | 0.015 | 1.35     | 0.08     | 0.16     | 0.3      | 1.9      |    |

*Per cent recovery.*

|            | Au.   | Ag.   | Cu.   | Pb.   | Zn.   | Fe.   | 80    |
|------------|-------|-------|-------|-------|-------|-------|-------|
| Heads..... | 100.0 | 100.0 | 100.0 | 100.0 | 100.0 | 100.0 | 100.0 |
| Cones..... | 75.0  | 94.5  | 82.3  | 90.4  | 74.5  | 18.5  |       |
| Midds..... | 4.0   | 2.4   | 2.2   | 3.2   | 11.5  | 10.5  |       |
| Tails..... | 17.1  | 3.1   | 15.5  | 6.4   | 14.0  | 71.0  |       |

Similar results were obtained when petro- 85 lastic cement was substituted for the air-blown-paraffin-base asphalt.

I claim:

1. The process of froth-flotation concentration which consists in agitating and 90 aerating a pulp of suitably ground material with a non-acid mineral-frothing agent consisting of mixed benzene-series hydrocarbons and asphalt, and separating the froth.

2. The process of froth-flotation concentration which consists in agitating and 95 aerating a pulp of suitably ground material with a non-acid mineral-frothing agent consisting of mixed benzene-series hydrocarbons and asphalt, separating the froth, agitating the remainder of the pulp with a further 100 quantity of mixed benzene-series hydrocarbons and asphalt, and separating a second froth.

3. The process of froth-flotation concentration which consists in agitating and 105 aerating a pulp of suitably ground material with a non-acid mineral-frothing agent consisting of mixed benzene-series hydrocarbons and asphalt, separating the froth, agitating the remainder of the pulp with a further 110 quantity of mixed benzene-series hydrocarbons and asphalt, and separating a second froth.

4. The process of froth-flotation concentration of an iron-bearing lead-zinc ore 115 which consists in agitating and aerating a pulp of the suitably ground ore with a non-acid mineral-frothing agent consisting of mixed benzene-series hydrocarbons and asphalt, separating a froth relatively rich in a 120 lead, agitating the remainder of the pulp, with a further quantity of mixed benzene-series hydrocarbons, and separating a second froth, relatively rich in zinc.

5. The process of froth-flotation concentration of an iron-bearing lead-zinc ore 125 which consists in agitating and aerating a pulp of the suitably ground ore with a non-acid mineral-frothing agent consisting of mixed benzene-series hydrocarbons and as- 130

phalt, separating a froth relatively rich in lead, agitating the remainder of the pulp with a further quantity of mixed benzene-series hydrocarbons and asphalt, and separating a second froth relatively rich in zinc.

6. The process of froth-flotation concentration which consists in agitating and aerating a pulp of suitably ground material with a non-acid mineral-frothing agent consisting of xylol carrying asphalt, and separating the froth.

7. The process of froth-flotation concentration which consists in agitating and aerating a pulp of suitably ground material with a non-acid mineral-frothing agent consisting of mixed benzene-series hydrocarbons carrying paraffine-base-petroleum-air-blown asphalt, and separating the froth.

In testimony whereof, I have affixed my signature to this specification.

JOHN W. LITTLEFORD.